

## UNITED STATES PATENT OFFICE

2,341,861

METHOD OF PROCESSING SWELLING COALS  
FOR USE IN BY-PRODUCT OVENS

Walter M. Fuchs, State College, Pa.

No Drawing. Application December 17, 1941,  
Serial No. 423,336

2 Claims. (Cl. 202—25)

The invention relates to a processed coking coal and to a method of decreasing the swelling pressure of coals.

One of the objects of my invention is to prepare a swelling coal for safe use in the manufacture of coke in byproduct ovens.

Another object of my invention is to treat a swelling coal with air of controlled moisture content in order to decrease its swelling power without impairing its coking quality.

Another object of my invention is to oxidize at relatively low temperature and pressure, as a pretreatment to coking, swelling coals of the size distribution used for composing carbonization blends.

Another object of my invention is to use pre-treated coals in blends with untreated coals, or other pretreated coals.

Other objects of my invention are set forth in the following description, it being understood that the above statement of the objects of my invention is intended to generally explain the same without limiting the same in any manner.

Likewise, I do not wish to be limited to the specific examples which are later given herein as illustrating embodiments of the invention, since numerous changes in procedure may be made without departing from the spirit of the invention.

The term swelling pressure of coal is used to indicate the fact that pressure against the oven wall is noted during carbonization. It has been recognized that swelling power, i. e., the property to develop swelling pressure, is common to all coking coals. At present, the term swelling coals is used for a group of coking coals which belong to the low- and medium-volatile group, exhibit a low or medium cakeability, and are found to develop excessive swelling pressure. However, it has been recognized that swelling pressure is not only dependent upon the nature of the coal but also upon the conditions of the coking operation, such as oven width and rate of heating. Control of swelling pressure has been greatly facilitated by a thermodynamic analysis of the phenomenon (J. Franklin Inst. 231, 103-119, 1941), and by the development of a satisfactory measuring device (Am. Gas Assoc. Meeting, May 1941, New York city). The measuring device permits to work with a coking chamber of variable width; the data obtained may be extrapolated to actual conditions.

It has been established that the swelling power can be decreased by weathering, addition of inert material, of chemicals (either organic or in-

organic), and the like. All these actions may be successful as far as mere decrease of swelling power is concerned. They result, however, as a rule in a simultaneous deterioration of quality of either coal or coke or both.

The same is noted upon treating coal with air, as suggested in various patents for diverse purposes. In U. S. Patent 1,993,198 (Wisner) it is stated "that finely crushed volatile coal in the range of 350 to 450° F. is in a rascant condition as regards oxygen, that is, it is free to be rapidly modified and conditioned for coking in ovens and carbonizing in retorts, for stopping sticking to container walls, and controlling expansion during the softening period of carbonization, for producing a denser and stronger product, and for shortening the process cycle, thereby contributing a new step to carbonization technology." To carry out the process, finely divided coal freed of surface moisture is treated for a time from 10 to 45 minutes with an amount of air varying from zero to 2000 cubic feet per ton of coal.

It is correct that under the conditions disclosed by Wisner a rapid modification of the coal occurs. But because of this rapidity of change the process is not applicable to swelling coals which do not possess a high cakeability and quickly loose their value as coking coals by such treatment. This is demonstrated by the following observations:

A swelling coal with 18% vol. matter ground to pass a 60 mesh sieve was treated at various temperatures for various lengths of time in a rotary furnace with a current of air. The effect of the treatment was followed by measurements of swelling pressure and by coke button tests. From 150° C. upward the swelling power decreased quickly. This, however, was accompanied by a rapid deterioration of coal quality. Coke buttons prepared at even intervals showed a steady decrease in strength. After a relatively short time, e. g., 60 minutes at 200° C. no coke button at all was formed, merely an incoherent residue was obtained. Hence, the Wisner process applied to low- and medium-volatile coals results in a serious deterioration defeating the purpose of decreasing the swelling power without impairing the coke forming properties.

In U. S. Patent 2,167,100 (Benezech) an improvement of coking coal is claimed by subjecting it to a predetermined limited degree of oxidation to reduce its cakeability. The process is carried out by storing the coal with only the air normally entrained in it, and aging the coal in

the bunker column for at least several days at a temperature from 130 to 160° C.

I have designed a process in order to decrease the swelling pressure of swelling coals by treatment with air, and yet avoid both the danger of deterioration attendant upon rapid oxidation, and the inconvenience inherent to an aging process extended over a period of several days. The process is based on the following observations:

1. In contrast to finely crushed swelling coal, swelling coal of commercial size distribution, e. g.,  $\frac{1}{2}$  inch slack, is not easily oxidized. A slack sample of coal with 18% volatile matter was studied under the conditions recorded for the -60 mesh sample. As shown by coke button tests, the coking properties were hardly impaired even after 10 hours of oxidation. Blends prepared by the use of oxidized slack samples showed a substantial decrease of swelling pressure, e. g., from 5 lbs. to 1.5 lbs. per square inch. However, difficulties were encountered in attempts to duplicate results closely.

2. Satisfactory duplicability of results, satisfactory diminutions of swelling power, and unchanged or even improved coking properties resulted from a treatment with air of constant humidity. Apparently, this factor has escaped attention in the prior art.

3. Optimum conditions of processing were determined by following the operation with the measuring device.

The application of these observations is illustrated by the following examples:

*Example 1.*—A  $\frac{1}{2}$  inch slack sample of a Pocahontas coal with 16.3% volatile matter was treated in a rotary furnace at 300° C. for three hours with a current of air that had been saturated with water vapor at room temperature; per ton of coal, 3300 cubic feet of air were

used. The processed coal showed a substantial decrease of swelling pressure and permitted obtaining of a coke with decreased porosity and increased strength.

5 *Example 2.*—A  $\frac{1}{2}$  inch slack sample of a Miller seam coal with 22.0% volatile matter was treated in a rotary furnace at 240° C. for one hour with a current of air that had been saturated with water vapor at 60° C.; per ton of coal, 1100 cubic feet of air were used. The processed coal showed a substantial decrease of swelling pressure without a noticeable decrease of cakeability.

I claim:

15 1. A method of processing swelling coals of commercial size distribution for use in byproduct ovens by treatment with air of a moisture content between 0.01 and 0.5 lb. of water vapor per lb. of dry air, the treatment to be effected prior to carbonization in the temperature range from 150° C. to 300° C. for such a period of time that the original swelling pressure is decreased to a value not exceeding 1.5 lb. per square inch of oven wall on the basis of the coal charge to be carbonized.

20 2. A method of processing swelling coals of commercial size distribution for use in byproduct ovens by treatment with air of a moisture content between 0.01 and 0.5 lb. of water vapor per lb. of dry air maintained by saturating the air with water vapor at the corresponding temperature between 10 and 75° C., the treatment to be effected prior to carbonization in the temperature range from 150° C. to 300° C. for such a period of time that the original swelling pressure is decreased to a value not exceeding 1.5 lb. per square inch of oven wall on the basis of the coal charge to be carbonized.

WALTER M. FUCHS.